

No. 756,173.

PATENTED MAR. 29, 1904.

I. P. LIHME.  
PRESERVED WOOD AND PROCESS OF PREPARING SAME.  
APPLICATION FILED JUNE 7, 1902.

NO MODEL.

Fig. 1.



Fig. 2.



WITNESSES:

W. A. Shunk  
George B. Riley

INVENTOR:

Iens P. Lihme

by his attorney,

Albert Dunn Lawrence

## UNITED STATES PATENT OFFICE.

IENS P. LIHME, OF CLEVELAND, OHIO, ASSIGNOR TO THE GRASSELLI CHEMICAL COMPANY, OF CLEVELAND, OHIO, A CORPORATION OF OHIO.

## PRESERVED WOOD AND PROCESS OF PREPARING SAME.

SPECIFICATION forming part of Letters Patent No. 756,173, dated March 29, 1904.

Application filed June 7, 1902. Serial No. 110,623. (No specimens.)

*To all whom it may concern:*

Be it known that I, IENS P. LIHME, a citizen of the United States of America, and a resident of Cleveland, in the county of Cuyahoga and State of Ohio, have invented certain new and useful Improvements in Preserved Wood and Processes of Preparing Same, (Case No. 3,) of which the following is a specification.

My invention relates to improvements in preserved wood and process of preparing same, and has for its object the production of wood adapted to withstand moisture, heat, the attacks of insects, and, in short, to render the treated wood as nearly impervious and unaffected by the elements as possible.

Zinc chlorid has long been recognized as an extremely efficient if not the best wood preservative known; but this has been coupled with the distinct disadvantage of the chemical's being quite readily dissolved from the pores of the impregnated wood when exposed to the action of the air and rain, thus leaving the wood entirely unprotected. It has accordingly ranked heretofore as a temporary preservative. The silicates, notably that of sodium, have likewise been resorted to for the purpose of fireproofing wood and have been proven extremely efficient, but are open to the same objection just mentioned. My present invention accordingly proceeds with the idea of combining the advantages of each of these two extremely efficient wood-preserving agents, while attaining practical permanence in the preservative effect secured.

Adverting briefly to my improved process and product, I may state, as introductory to a more extended description thereof, that the process preferably consists in first effecting approximately the complete filling of the pores or saturation of the treated wood with a solution of zinc chlorid and thereafter subjecting the same to the action of a silicate solution, as sodium silicate, the use of vacuum and pressure being resorted to in order to obtain the desired impregnation. Under this treatment it will be found that the body of the wood is thoroughly impregnated with the

first-named salt, constituting an excellent preservative, while the exterior portion of said wood contains in its pores a superficial crust 50 of varying depth, composed of silicate of zinc, which is both insoluble and fireproof and closes in the soluble chlorid contained in the interior of the wood.

My invention may be more readily explained 55 by referring to the accompanying drawings, wherein—

Figure 1 illustrates in somewhat diagrammatic manner apparatus adapted for practicing my invention, and Fig. 2 shows in cross-section a log or railroad-tie and a board after their treatment in accordance with my improved process.

In practicing my process a hermetically-closed chamber is required, preferably of such 65 capacity that a large charge of wood may be readily inserted for treatment and easily removed therefrom.

In the drawings I have indicated a large chamber *a*, capable of being securely sealed 70 by a door *b* after the car *c*, carrying the wood *d* to be treated, has been pushed within the chamber. Beneath the rails are shown steam-coils *e* for inducing a high temperature within the treating-chamber. A vacuum-pump *f*, 75 with its gage *f'*, and a fluid-pump *g*, with its corresponding pressure-gage *g'*, are connected with the said chamber *a*. A pressure-equalizer *h* also is associated with the said chamber, the same having a movable weighted head *h'*, 80 adapted to be raised in its cylinder upon the increase in the pressure within the chamber beyond a given point. Upon introducing the wood within the chamber it is first subjected to a dry heat of about 200° by admitting steam 85 to the coils *e*, which heating is continued until the wood has become thoroughly dried. The vacuum-pump *f* is then put in operation until the gage *f'* remains substantially constant. The valves *i* *k* in pipes *i* *k* are then 90 opened, the latter pipe connecting with the tank containing a zinc-chlorid solution, whereupon the treating-chamber is flooded with the said solution of zinc chlorid. Valve *i'* is then

closed and pump  $g$  is set in operation and a pressure of approximately two hundred pounds to the square inch is secured, which pressure is maintained ordinarily for five or six hours. It may be well here to observe that the details of the treating process or operation vary considerably, depending upon the kind and condition of the wood under treatment, so that only general statements can be made which are applicable to average circumstances. This high pressure is continued until the wood has become thoroughly impregnated with the zinc chlorid, this operation being greatly facilitated by the previous exhaustion of the air, after which the solution is pumped out of the chamber and into the containing-tank. (Not shown in the drawings.) Valve  $k'$  is thereupon closed and valve  $l'$  is opened to permit the solution of sodium silicate to be pumped through pipe  $l$  into the treating-chamber. As before, the solution is maintained under a high pressure until the desired impregnation with silicate takes place. Treatment under two hundred pounds pressure for five or six hours will commonly suffice. By reason of the previous impregnation, however, it will be found that the formation of zinc silicate in the exterior portions of the wood through the combination of the two salts will clog or check the reaction more and more and cause the formation of an impervious layer or superficial crust within the pores of the wood. Depending again upon the kind of wood and conditions of treatment, this layer will be of greater or less thickness—say, from one-eighth to three-quarters of an inch—but will be found sufficient to permeate the wood to form an effective exterior protection therefor. After withdrawing the silicate solution from the chamber steam may be admitted to the coils to effect the rapid drying of the treated wood or the car may be removed from the chamber, permitting its recharging while the treated wood is allowed to dry naturally before making use of it.

It is scarcely necessary to state that proper precautions should be taken to insure the free access of the separate solutions to all of the wood under treatment. The strengths of the solutions used ordinarily will be from five per cent. to ten per cent., no precise general directions being practicable, however, since in

this matter the process depends as well upon the kind and condition of the wood treated.

This process is particularly valuable in preserving railroad-ties, and in Fig. 2 is shown in cross-section a tie after being subjected to my above-described process, as well as a similar view of a board likewise treated. Each will be found to have a central portion  $x$  thoroughly impregnated with the preservative zinc chlorid and an external zone or permeating-crust  $y$  of insoluble zinc silicate. This latter—viz., the protective crust of zinc silicate—is of course perfectly insoluble, impervious to water, and relatively unaffected by fire or extremes of heat and cold and the attacks of insects. Hence it forms an ideal protection for the body of wood inclosed thereby.

Having now described my invention, I make claim to the following:

1. The herein-described process for treating wood, consisting in effecting its thorough impregnation with zinc chlorid and thereafter subjecting the wood to the action of a soluble silicate, preferably sodium silicate, whereby a layer or superficial crust of zinc silicate is formed in the exterior portions of the wood, substantially as set forth.

2. The process substantially as herein described, for preserving railroad-ties and the like, which consists in effecting the thorough impregnation of the wood with a zinc-chlorid solution by means both of vacuum and high pressure, and then subjecting said wood to a solution of a soluble silicate, preferably sodium silicate, under pressure whereby zinc silicate is precipitated in the pores of the wood to a moderate depth.

3. The product of the herein-described process, comprising wood, such as railroad-ties, thoroughly impregnated substantially throughout its interior with zinc chlorid, and its exterior portions permeated with a protective layer of zinc silicate, substantially as set forth.

Signed by me at Cleveland, Ohio, in the presence of two subscribing witnesses, this 26th day of May, A. D. 1902.

IENS P. LIHME.

Witnesses:

GEORGE B. RILEY,  
ALBERT LYNN LAWRENCE.